

## UNITED STATES PATENT OFFICE

2,206,369

## FOUNDRY SAND BINDER

Harold K. Salzberg, Pittsburgh, Pa.

No Drawing. Application April 29, 1938,  
Serial No. 205,123

12 Claims. (Cl. 22—188)

This invention relates to foundry sand binders, methods of using the same, and to products made by the foundry use of such binders.

In the art of sand-casting metals, cores and molds are employed made of foundry sand bonded with a suitable binder and baked in the desired shape. A great many metal castings are made by pouring molten metal into molds made of sand, into which have been set preformed cores to provide openings and cavities in the casting of the requisite design. The molten metal when poured into these molds flows against inside and outside surfaces of sand, and usually surrounds the surfaces of the cores.

15 These cores and frequently also the molds are made by ramming a moistened mixture of foundry sand containing a small proportion of a binder into a core box or around a pattern. The molded sand and binder mixture may be left in the wet or green condition after shaping, but more often 20 the core or mold thus formed is baked in an oven, or otherwise dried, to provide the shaped article with the necessary strength to enable it to maintain its shape during handling, and during pouring of the metal.

25 The foundry sand binder employed should readily mix with sand and should not cause the wet sand to stick to the core box or pattern. It is also desirable to use a binder which provides the wet sand originally with some strength commonly referred to as "green bond strength." Where the core is to be dried or baked, the binder must be capable of withstanding oven temperature and must be strong enough to hold the grains of sand in the desired form in the dry state, without employing more than a very small percentage of binder in proportion to the amount of sand used. Too large a quantity of binder might produce excess "gassing" when the casting is poured. In addition, the binder should be selected so that 30 it will burn out of the sand at the proper rate during the casting operation and it should not leave the sand in and around the formed casting in such a state that it is difficult to remove from the metal.

45 One object of my invention is to provide an economical foundry sand binder which satisfactorily meets the requirements of the foundry art to a high degree.

50 Another object of this invention is to provide an economical foundry sand binder which produces high strengths in a baked sand core, even when used in extremely small amounts in proportion to the sand.

55 A further object of this invention is to provide

baked sand foundry molds and cores having the requisite properties developed by such foundry sand binders.

Another object is to provide an improved core paste for foundry use. Other objects will be 5 explained and will be apparent from the following description of my invention.

Seed meals, particularly those seed meals high in available protein, are inexpensive materials which would be very valuable alone as foundry 10 binders if they possessed a higher binding value for sand. I have discovered that such seed meals may be greatly improved in their binding properties by the addition of a suitable conditioner or modifying agent. Outstanding among these modifiers are the water soluble oxalates, borates, and fluorides. The metaphosphates and sulphates also have a very advantageous effect, and such phosphates, carbonates, and chlorides as trisodium phosphate, soda ash and sodium chloride 20 produce substantial improvements in the action of the seed meals as foundry sand binders. The modifiers employed are preferably the water soluble salts. The improved core binders of my invention may be employed in relatively small 25 amounts with the sand, thereby preventing excessive gassing during pouring of the castings. The amount of binder used will depend on the particular foundry requirements and will generally be about 1 to 2% by weight of the sand. 30

One of the particular advantages of my invention is the fact that these modifiers may be employed to good effect with the spent or by-product seed meals, i. e., the seed meals remaining after commercial extraction of the oils which these oil 35 bearing seeds contain in their original state.

By the term "seed meals" as used herein, I intend to include those seed meals which are relatively high in protein, such as soy bean, peanut, pea, castor bean, cottonseed and linseed meal, as 40 distinguished from the flours or meals of corn, wheat, barley, oats, and the like. The meals may either contain all of the original oil or have part or all of the oil extracted therefrom. For economic reasons, the latter will be preferable. 45

The foregoing seed meals useful for purposes of my invention have a protein content of more than about 20% on an oil free basis.

I prefer to employ those seed meals which have not been subjected to high temperatures, because 50 this reduces the quantity of available water soluble protein in the final product. A seed meal best suited for purposes of my invention is one that contains at least about 35% of the total protein content as water soluble protein, and that 55

has not been subjected to a temperature materially above 135° F., as occurs in the hot pressing of certain seed meals to extract oils therefrom.

The seed meals employed are also preferably finely divided; in general, the finer the seed meal is ground, the higher core strength may be obtained by the use of the modified seed meal as a core binder.

With regard to the conditioner or modifying agent employed, I prefer to use the water soluble salts, and have found that the best results are obtained with an oxalate, or a borate such as borax. For example, the transverse breaking strength of standard baked test bars made with 15 foundry core sand and 1% by weight of a binder comprising a seed meal modified by sodium oxalate is more than double, and in some cases more than three times the strength of test bars made with the same proportion of the same seed 20 meal alone.

The proportion of the modifier or conditioner added to the seed meal should be adjusted according to the grade of seed meal and the particular modifier employed. With a low grade 25 seed meal, in general, more of the modifier is required. When a high grade seed meal is employed, i. e., a seed meal from which the oil has been extracted by a solvent leaving a higher proportion of water soluble protein, a smaller proportion of the oxalate, preferably not more than 30 about 6%, is employed. With such high grade meals, the maximum effect of the oxalate appears to be obtained using about 4% of an oxalate based on the weight of the seed meal. 35 As the proportion of modifier is increased beyond the point of maximum effect, the strength of baked cores made with the core binders progressively decreases. The other salts are less effective than the oxalate and produce their maximum effect when employed in somewhat larger amounts than the oxalates. For example, sodium metaphosphate used with some seed meals may be required in the proportion of 11% to produce its maximum effect. The modifiers of my invention 45 may be employed effectively in amounts up to about 12% of the seed meal.

Other improvements effected by using modified seed meals in accordance with my invention over the use of seed meals alone are the great increases 50 obtained in dry tensile strength, resistance to abrasion, and green bond strength in the sand cores. Any suitable foundry sand may be employed in accordance with my invention.

The improvements obtained by using a mixture 55 of a seed meal with a modifying agent as a core binder are not limited to the use of the seed meal and modifier alone, but these improvements also are obtained when the seed meals are used in sand containing other binders, such as flour, 60 waste sulfite liquor, molasses and the like. The presence of these other ingredients does not exclude the enhancing effect of the oxalate or other modifier on the seed meal employed.

A particularly advantageous and unique mixture 65 of binders is a core binder comprising a mixture of milk solids with a seed meal and a modifier in accordance with this invention. The combination of a seed meal and milk solids with a modifying agent such as sodium oxalate is 70 unusual because such a mixture is capable of producing higher core strengths in baked sand foundry cores than the additive sum of strengths obtained by using comparable quantities of the seed meal and modifier and of the milk solids 75 and modifier alone. This unusual effect is ob-

tained in a modified mixture of milk solids and seed meals in virtually any proportions. The mixture may consist principally of milk solids or principally of the seed meal, or it may be a mixture of approximately equal parts of these ingredients together with the modifier. This makes it possible to provide an extremely valuable core binder of very intensive effect containing a relatively inexpensive seed meal. The following are 10 good examples of such mixtures, the proportions being in parts by weight.

|                       | I  | II | III |
|-----------------------|----|----|-----|
| Skim milk powder..... | 80 | 40 | 20  |
| Soy bean flour.....   | 20 | 60 | 80  |
| Sodium oxalate.....   | 4  | 5  | 6   |

The amount of modifier used with these mixtures should be based on the total weight of seed meal and/or milk solids instead of on the quantity of seed meal alone. By "milk solids" I mean either dried milk solids such as skim, partially skimmed or whole milk powders, the corresponding fluid milk products in a natural 25 or condensed state, or mixtures thereof.

I prefer to employ a dry mixture of the foregoing ingredients, although the modifying agent may be added to the sand before or after the seed meal flour is added, or the modifying agent 30 may be added to the water used in tempering the sand, or with water which is swabbed or sprayed on the formed core or mold before it is baked.

While I do not wish to be limited by any theory of the operation of these modifying agents, I believe that the nature of the action on the seed meals is a peptizing of the protein content 40 thereof. The action of the modifying agents on the milk solids may be of a different or of the same character.

In general, the strengths of the baked core produced using a mixture of milk solids with a seed meal and modifying agent are higher, the greater the proportion of milk solids employed. 45 The particular proportion of these ingredients may be adjusted depending upon the strengths desired and the costs of the two ingredients.

A small amount of the order of 1 to 3% of an oil, such as a low viscosity mineral oil, may be 50 added with good effect to a core binder in accordance with my invention. This has some value in eliminating dusting of the product and removing stickiness of the sand and core binder mixture after it has been moistened. The workability of the moistened sand and binder mixture 55 is also improved by this addition.

The core binders of this invention may also be employed in combination with a core oil where free flowing characteristics of the sand are desired, as in the use of automatic core making machines. Under these conditions, I prefer to add a salt of nickel or iron to the mixed core binder in order to take full advantage of the greatly increased strengths obtained by the core binders of my invention. The use of a mixture, for example, of 1% of an ordinary core oil and 1/2 of 1% of a binder in accordance with my invention produces a free flowing sand. The ingredients of my seed meal binders however, have an inhibiting effect on the drying of the core oil, thereby resulting in lower core strengths than should be obtained with such mixtures. The addition of a small percentage of an iron or nickel salt which may be organic or inorganic, oil or water soluble 70

eliminates this inhibiting effect. The salts of these metals appear to have some catalytic action and may be included in any core binder of my invention whether or not it is actually used with a core oil, since they do not substantially injure the strength of such binders when used in small amounts of the order of 5% or less. If desired, the oxalate or other modifying radical may be included in the iron or nickel salt, although only such combinations as are water soluble should be employed. Ferric oxalate or ferric ammonium oxalate are examples of useful salts of this nature.

A preferred composition of core binder in accordance with my invention is as follows:

| Parts by weight               |     |
|-------------------------------|-----|
| Roller dried skim milk powder | 40  |
| Soybean flour                 | 60  |
| Sodium oxalate                | 6   |
| 20 Preservative (Dowicide)    | 1/2 |
| Mineral oil                   | 2   |
| Ferric sulfate                | 3   |

The core binders of my invention, particularly those including milk solids, also are useful as a core paste. The above composition, or other modified seed metal binders, may be used as a paste directly upon admixture with water for sticking parts of cores together. The use of this material as a core paste is greatly enhanced however, by the addition of some clay or other finely divided relatively inert material, such as silica flour. The inert material may be employed in proportions of about 2 to 4 parts of inert material to one part of modified seed meal, with or without milk solids.

A preferred composition of core paste using a modified seed meal in accordance with my invention is as follows:

| Parts                           |       |
|---------------------------------|-------|
| 40 Silica flour (finely ground) | 75    |
| Skim milk powder                | 15    |
| Soybean meal flour              | 10    |
| Sodium oxalate                  | 1 1/4 |
| 45 Ground rosin                 | 5     |
| Borax                           | 1     |
| Mineral oil                     | 1     |

In such a paste, the inert material, which may be clay or silica flour, lends heat resistance to the joint, providing higher joint strength during and after pouring of the metal. The addition of rosin improves the water resistance of the joint and makes the paste formed with water a little thicker. The sodium oxalate and borax act, as previously described, to improve the effect of the skim milk powder and seed metal. The mineral oil serves to reduce the dustiness of the dry paste and also provides a smoother product for brushing.

60 When employing the composition of my invention as a core paste, about two parts of the solids may be mixed with one to two parts water. The particular amount of water will probably vary, depending on the particular use for the paste.

65 A highly fluid paste is desired when ease of application is required, as when mechanical means are employed for applying the paste. On the other hand, a very thick putty may be needed especially when sealing the core joints. A wide range of consistency of paste is possible by merely regulating the ratio of water to dry material.

I have also found that the foundry sand binders of my invention, and more particularly binders containing finely divided inert material such as the product obtained by using the above for-

mula for core paste are useful as a base for coatings for cores and molds. Such coatings are commonly referred to as "washes." A thin suspension of the material in water, for example, one pint of dry paste solids to two pints of water, can be used to advantage in brushing or swabbing cores or molds. The purpose of such coatings is to provide a surface more resistant than the bare sand surface to the heat of the metal, and their use makes for a smoother finish on the casting. The wash prepared with the materials of the above mixture exhibits the effect of the chemicals on the mixture of milk solids and seed meal flour in providing a hard, non-chalky, strongly adherent coating.

The purpose of the borax in this formula becomes twofold when the suspension is thin enough for use as a wash. In addition to improving the adhesive power of the mixture of milk powder and seed meal flour, borax also acts as a suspending agent for the silica particles, thus overcoming the natural tendency of the silica to settle out and to form a hard sediment when the suspension is allowed to stand undisturbed for long periods of time. For this reason, I prefer to employ borax, with or without some other modifying agent, when the foundry binders of my invention are used with a thin suspension of finely divided inert material such as silica.

By the term "foundry sand binder" I intend to include such foundry uses for the products of my invention as core binders, core pastes, and core or mold washes for which these products are particularly well suited.

The terms and expressions which I have employed are used as terms of description and not of limitation, and I have no intention, in the use of such terms and expressions of excluding any equivalents of the features shown and described or portions thereof, but recognize that various modifications are possible within the scope of the invention claimed.

I claim:

1. A foundry sand binder comprising finely divided seed meal containing more than about 20% protein on an oil free basis, milk solids, and an effective amount up to about 12% of the combined weight of milk solids and seed meal of a soluble salt of the class consisting of oxalates, borates, fluorides, phosphates, sulfates, carbonates and chlorides.

2. A foundry sand binder comprising a finely divided seed meal of the group consisting of soy bean, peanut, pea, castor bean, cottonseed, and linseed meals, milk solids, and a small amount not more than about 10% by weight of a water soluble oxalate.

3. A foundry core binder comprising finely divided soy bean meal, milk solids and a water soluble oxalate in the proportion of about 2 to 6% of the total weight of soy bean meal plus milk solids.

4. A foundry sand binder comprising finely divided seed meal containing more than about 20% protein on an oil free basis, a small amount of a salt of a metal of the group consisting of iron and nickel, and an effective amount up to about 12% of a water soluble salt of the class consisting of oxalates, borates, fluorides, phosphates, sulfates, carbonates and chlorides.

5. A foundry sand binder comprising finely divided seed meal containing more than about 20% protein on an oil free basis, milk solids, a small amount of a salt of a metal of the group consisting of iron and nickel, and an effective

amount up to about 12% of a water soluble salt of the class consisting of oxalates, borates, fluorides, phosphates, sulfates, carbonates and chlorides.

5 6. A foundry sand binder comprising finely divided seed meal containing more than about 20% protein on an oil free basis, milk solids, core oil, a small amount not greater than about 5% of an iron salt, and an effective amount up to about 10% of a water soluble oxalate.

10 7. A foundry core paste composition comprising principally finely divided inert material, a smaller proportion of a finely divided seed meal containing more than about 20% protein on an oil free basis, milk solids, and a water soluble oxalate in an amount not substantially greater than 10% of the combined amount of milk solids and seed meal.

15 8. A foundry core wash composition comprising principally finely divided inert material, finely divided seed meal containing more than about 20% protein on an oil free basis, milk solids, and a small amount of borax.

20 9. The method of preparing material for foundry use comprising working into a substantially uniform plastic mixture finely divided inert material, seed meal containing more than about 20% protein on an oil free basis, milk solids, and a water soluble salt of the class consisting of 25 oxalates, in an amount not greater than about 30

10% of the total weight of seed meal and milk solids.

10 10. The method of preparing material for foundry use comprising working into a substantially uniform plastic mixture finely divided inert 5 material, seed meal containing more than about 20% protein on an oil free basis, milk solids and a water soluble oxalate, the oxalate being present in an amount of about 2 to 6% of the combined weight of seed meal and milk solids.

10 11. A process of making a foundry core comprising preparing a moistened mix of foundry sand and a binder comprising finely divided seed meal containing more than about 20% protein on an oil free basis and milk solids modified by 15 a water soluble salt from the class consisting of oxalates, borates, fluorides, phosphates, sulfates, carbonates and chlorides, shaping said mix to form a core and baking said core.

15 12. A baked foundry core comprising foundry sand held together in a coherent mass by a binder resulting from baking a moistened foundry sand mix containing finely divided seed meal containing more than about 20% protein on an oil free basis and milk solids modified by a water 25 soluble salt from the class consisting of oxalates, borates, fluorides, phosphates, sulfates, carbonates and chlorides.

HAROLD K. SALZBERG. 30